

April 13, 1926.

1,580,647

G. D. BRECK

PROCESS FOR TREATING FERROUS METAL TO PREVENT CORROSION

Filed Feb. 25, 1921



Inventor  
George D. Breck  
By Harold Elio Smith  
Atty.

## UNITED STATES PATENT OFFICE.

GEORGE D. BRECK, OF CLEVELAND, OHIO.

## PROCESS FOR TREATING FERROUS METAL TO PREVENT CORROSION.

Application filed February 25, 1921. Serial No. 447,772.

*To all whom it may concern:*

Be it known that I, GEORGE D. BRECK, a citizen of the United States, residing at Cleveland, in the county of Cuyahoga and State of Ohio, have invented a certain new and useful Improvement in Processes for Treating Ferrous Metal to Prevent Corrosion, of which the following is a full, clear, and exact description, reference being 10 had to the accompanying drawings.

This invention relates to the treatment of ferrous metal for the purpose of preventing corrosion. The fundamental object is the provision of a tube or pipe so treated, either internally or externally or both, as to be usable for the economizers of steam boilers, or feed water heaters, since it is well known that ordinary steel pipes become corroded very rapidly when put to this use, 15 interiorly because of the air, gas, or chemical substances dissolved in the water, and exteriorly because of the acid deposit condensed thereon from the furnace gases, or surrounding atmosphere. However my invention is not limited to this use inasmuch as a tube which has sufficient resistance to corrosion for the purpose indicated is also 20 usable in numberless other relations in the arts, and a process which will produce such a tube is equally applicable to the production of ferrous metal articles for a great variety of different technical purposes, whether subjected to hot, cold, wet, dry, acid, alkaline, climatic or other injurious 25 conditions; and I hereby declare my purpose to claim and secure my invention for all uses to which the same may be applicable.

Subsidiary objects of the invention are the provision of a method of treating ferrous metal which is applicable to commercial, hot-rolled or forged, steel products and of all manner of cross section; which can be employed without departing from the established commercial methods of steel rolling; which is applicable to steel in the ductile state and is not restricted to castings as in the case of many non-corrodible compositions heretofore suggested; which does not materially decrease the flexibility or ductility or other physical properties of the material; which can be performed with commercial and inexpensive materials; the provision of certain new and improved articles and compositions of matter; while other objects and advantages of the invention will

become apparent as the description proceeds.

The essence of my invention resides in the superficial application to a ferrous metal while rendered plastic by heat, of a protective metal or alloy in finely divided form, and immediately incorporating the same into the ferrous metal by mechanical working such as rolling or forging, the temperature of the ferrous metal being below the melting point of the added material. I do not restrict myself to the use of any one metal or alloy excepting that the applied material must be one which will alloy with the ferrous metal with the production of a solid solution alloy forming a coating which is highly resistant to corrosion and is so closely adherent as not to scale or peel off; and further that it should possess a sufficiently high melting point to withstand all ordinary vicissitudes of use. These considerations alone exclude the employment of material consisting of or containing any large proportion of such ingredients as tin, lead, zinc, arsenic, antimony, bismuth, cadmium, or the like low melting-point metals. The material which I specially prefer is chromium or an alloy thereof, such as ferrochrome, or a mechanical mixture of finely divided chromium and iron; silicon also can be used to advantage in many cases, especially in association with other materials such as iron, chromium or aluminum. All these materials are characterized by the production of an impervious, adherent, insoluble alloy. Thus a commercial ferrochrome containing a rather large percentage of silicon affords the desired chemical advantages together with the physical property of being not unduly difficult to pulverize. Also the mixture of finely divided iron and chromium which is produced when chromite ore is reduced at temperatures below the melting point of iron or chromium, forms a very convenient material.

This material, mixed if desired with a suitable fluxing compound, is sprinkled on the surface of the white-hot blank, slab or billet just prior to its passing through the rolling mill, whereupon the pressure causes a true alloying of the ingredients even though the temperature be not sufficiently high to produce true fusion of the applied materials. In fact it is better not to have fusion of these materials since with fusion they become mobile and tend to segregate.

into drops and are removed by the rolling or forging operations whereas if fusion is avoided they remain in place. Before applying this treatment I preferably roll or 5 forge the metal sufficiently toward its finished dimensions so that the subsequent operations shall not serve to destroy the applied coating, reheating if necessary just prior to applying the powdered or granular 10 material. Also the nature of the operation first performed after such application is preferably one which does not greatly change the shape of the metal section but only incorporates the added material intimately 15 therewith, although this is generally attended with a decrease in the thickness of the blank accompanied by a corresponding spreading. After the coating is thus fixed in place the article can be repeatedly rolled or 20 forged, the surface layers expanding with the body parts throughout a considerable range of manipulation. Thus for example the blank may be circled into the form of a tube, having the coating either inside or 25 outside, or may be rolled into an I beam or other desired cross-section. In case it be desired to coat both sides I effect this by inverting the billet immediately after it has 30 passed through the first rolls, apply a similar coating of powdered material upon its opposite side and immediately re-roll the same, the smallest possible time being permitted to elapse between the two treatments so as to avoid unnecessary cooling.

35 In the drawings accompanying and forming part of this application Fig. 1 is a perspective view showing diagrammatically the performance of my invention; Figs. 2, 3, and 4 illustrate the simultaneous extension of 40 both coating and body upon working; Fig. 5 is a cross-sectional view of a tube having the described coating on its outer surface; Fig. 6 is a cross-sectional view of a blank having the described coating on both surfaces; Fig. 45 7 illustrates a tube having the described coating on both surfaces; and Fig. 8 is a cross sectional view of an I beam treated as herein described.

Describing the drawings by reference 50 characters, 1 represents a white-hot, steel or iron, sheet or billet, and 2-2 the rolls between which the same is passed, same being of any material known and used for that purpose, such as chilled cast iron, 3 represents the coating of applied pulverized material prior to the rolling and 4 represents a mechanical device of any suitable type 55 adapted to shower the material upon the entire surface of the metal in a uniform layer of the desired thickness. 5 illustrates the body and 6 the coating of the resulting sheet or plate. When made into tube form the same is circled and subsequently seam welded in the usual manner along the longitudinal line 7-7. In case of a hot rolled 60

tube the coating can be applied during the rolling process and a seamless tube secured with the non-corrodible surface I have described. 8 indicates a preheating device such as a gas burner which may be used if 70 desired. My improved compound metal articles are useful not only in connection with boilers and their accessories, but also in bridges and structural works exposed to climatic rusting; to furnaces, stove parts, 75 and metallurgical appliances exposed to high temperature corrosion; to various purposes where chemical corrosion is encountered; and in numerous other situations.

It will be understood that I do not restrict myself to the operation of rolling as the sole means of incorporating the powdered ingredients with the ferrous metal but have merely illustrated this as a type of mechanical working which involves pressure 85 and which can also be relieved by such other steps as forging or hammering; also that I do not restrict myself to steel, since wrought iron, charcoal iron, and other varieties of ferrous metal can be treated in this way, and 90 also such special alloys as nickel, steel, vanadium steel, and the like; I do not restrict myself to any particular degree of fineness of the applied coating, nor to any shape of finished article, and generally that I do not 95 restrict myself in anywise except as specifically set forth in the annexed claims.

Having thus described my invention what I claim is:

1. The process of producing non-corrodible metal elements which contains the steps of heating a slab or sheet of ferrous metal to a high temperature short of melting, covering the same with a superficial coating of a finely divided metallic substance which consists largely of chromium, and immediately rolling said slab or sheet while it is still plastic to the desired shape and size whereby said metallic substance is incorporated with the ferrous metal. 100

2. The process of producing an incorrodible article which contains the steps of heating a steel slab or blank to a temperature at which the same is plastic, applying to the surface thereof a superficial uniform layer 115 containing finely divided metallic chromium or an alloy thereof, incorporating such coating into such slab or blank by mechanical pressure, and subsequently reducing the slab or blank to finished form by repeated 120 rolling operations.

3. The process of treating ferrous metal to prevent corrosion which contains the step of rolling pulverized ferro chrome into the surface thereof at white heat. 125

4. The process of rendering steel incorrodible which contains the step of rolling into the surface thereof at white heat a finely divided metallic substance which contains 130 chromium.

5. The process of producing an incorrodible article which contains the steps of rolling pulverized ferro chrome mechanically into the surface of a white hot billet of ferrous metal and subsequently continuing the rolling until the desired shape is obtained and the applied coating is expanded so as to cover such shape. 25
6. The process of making an incorrodible tube which contains the steps of first rolling powdered ferro chrome into a flat, white-hot billet of ferrous metal, afterwards circling the resultant sheet into tubular form and welding the edges together longitudinally. 30
7. The process of making an incorrodible tube which contains the steps of heating a steel blank to a temperature of plasticity, covering the same with a finely divided metallic substance, which when alloyed pro- 35
- duces an impervious adherent, insoluble coating which is infusible at the temperature of such blank, incorporating such substance into said blank by mechanical pressure, expanding such blank into a sheet by pressure, and afterwards circling said sheet into a tube and welding the edges of the sheet together.
8. As an article of manufacture a hot rolled ferrous metal section having a superficial coating of chromium alloy formed thereon in situ. 30
9. A noncorrodible tube made of hot rolled ferrous metal having its inner surface coated with an unbroken adherent superficial alloy containing iron and chromium. 35

In testimony whereof, I hereunto affix my signature.

GEORGE D. BRECK.